

Feb. 8, 1966

CHUNG LIAO FENG

3,234,055

METHOD OF UNIFORMLY HEATING METAL PIECES

Filed Nov. 6, 1962



INVENTOR.  
CHUNG LIAO FENG  
BY *E. Welford Smart*

ATTORNEY.

3,234,055

METHOD OF UNIFORMLY HEATING  
METAL PIECES

Chung Liao Feng, Horsham, Pa., assignor to Selas Corporation of America, Dresher, Pa., a corporation of Pennsylvania

Filed Nov. 6, 1962, Ser. No. 235,751

3 Claims. (Cl. 148—13.1)

The present invention relates to a method of heating metal, and more particularly to a method of uniformly and rapidly heating metals having different surface conditions or a low surface emissivity.

In the heating of various metals, such as aluminum and brass for example, difficulty is encountered in bringing various pieces to the same temperature within the same time. This is due in large part to the varying emissivity of the surface of the pieces to be heated. Small pieces or slugs of aluminum or brass are prepared for hot working, such as forging, and stored until such time as they are needed. During the storage period the surface condition of the various slugs will alter appreciably, some being quite tarnished and others bright. When placed in a furnace to be heated, those slugs with tarnished surfaces will heat faster, or to a higher temperature in a given time, than those having bright surfaces. This is due to the different surface emissivity of the different pieces. The result is that it is difficult, if not impossible, to heat slugs of this type to an optimum forging temperature on a production line basis.

It is an object of the invention to coat uniformly the surfaces of a plurality of slugs as they are moving through a furnace so that they will be heated uniformly.

It is a further object of the invention to darken the surface of a bright metal object so that it will absorb heat more rapidly than would otherwise be the case.

In practicing the invention, slugs are moved one after the other through a furnace chamber having such a temperature and atmosphere that carbon is deposited uniformly over the surface of the slugs. The so-coated slugs then having a uniform surface appearance are moved into a heating zone of the furnace to be brought up to temperature. Since each slug then presents a similar surface to the furnace, they will be heated to substantially the same temperature in the same time. In addition, the dark coating of the carbon increases the speed of heating of slugs that were bright when moved into the furnace. The carbon coating disappears when the heated slug is removed from the furnace.

The various features of novelty which characterize my invention are pointed out with particularity in the claims annexed to and forming a part of this specification. For a better understanding of the invention, however, its advantages and specific objects attained with its use, reference should be had to the accompanying drawings and descriptive matter in which I have illustrated and described a preferred embodiment of the invention.

In the drawings: FIG. 1 is a view, in section, of one type of furnace that may be used to carry out the invention, and

FIG. 2 is a section taken on line 2—2 of FIG. 1.

Referring to the drawings, there is shown a furnace 1 having a floor 2 and end walls 3 and 4. The furnace is divided by a partition 5 into a pair of chambers 6 and 7. The end walls and the partition are provided with openings 8 that are shaped to conform with and closely encircle the work pieces as they are moved through the furnace on an endless conveyor belt 9. This belt passes over and is driven by pulleys 11 and 12, and is provided along its length with a plurality of sockets 13 into which the work pieces, shown herein by way of example only

as cylindrical slugs, 14 are received. The slugs can be placed on the sockets either manually or automatically and fall from the sockets down a discharge chute 15 to a work station, such as a forge, as the belt passes around pulley 12.

5 The chambers 6 and 7 are heated by burners 16 which may be of any conventional type, either flame or radiant, to the desired temperature. Fuel supplied to the burners is regulated by valves 17 which may be controlled manually or automatically in any conventional manner. The bottom or floor of chamber 6 is provided with a pair of openings through which the branches of a pipe 18 extend. This pipe is used to supply raw gas to the chamber with the supply being regulated by a valve 19.

10 15 The gas is supplied through the floor so that it will be closer to the portion of the chamber through which the pieces to be heated are moved.

In carrying out the method, the first furnace chamber 6 is heated by burners 16 to a temperature at least equal 20 to that at which the fuel gas being used will crack. If the gas is natural gas, for example, the temperature of chamber 6 will be at least 1500° F. The fuel supply to burners 16 is preferably stoichiometric, and in any event the products of combustion will be substantially neutral. 25 Gas is introduced into the bottom of chamber 6 through pipe 18. This gas is regulated by valve 19 until the atmosphere in the chamber has at least an equivalence ratio of 1.88 for the gas being used. With such conditions the excess gas will crack so that free carbon is produced in the furnace chamber.

30 The slugs, or other work pieces to be heated, are placed manually or automatically on fixtures 13 and moved at a constant speed through the furnace. The pieces being heated are normally at ambient temperature, or in any 35 event less than 300° F., as they move into the furnace. Because of their relatively cool temperature, the free carbon in the furnace chamber will immediately start to precipitate or be deposited in an even coating over the entire exposed surface of the piece, and each piece will be completely coated by the time the piece reaches 150° F. Belt 9 is moved at such a speed with relation to the length of chamber 6 that the pieces will reach at least this temperature before they enter chamber 7. The carbon forms a 40 uniform, thin, dark coating on each piece regardless of its original surface condition or color. Thus, the emissivity of the surface of each piece is substantially the same and for bright pieces is increased.

45 Chamber 7 is heated to a temperature dependent upon the final temperature of the work, but will ordinarily be 50 in the neighborhood of 2400° F. At this temperature the walls of the chamber will be incandescent so that a large percentage of the heating of the pieces will be by radiant heat, with the remainder being by convection from the burner gases. The absorption of radiant heat depends upon the emissivity of the surface of the piece being heated. A piece having a bright surface or one of low 55 emissivity requires a longer time to be heated to a given temperature than a piece with a dull surface. Since each 60 of the pieces has been coated so that it presents the same dull surface to the furnace, each piece will be heated substantially to the same temperature by the time it reaches the exit of the furnace. In addition, those pieces that originally had a bright surface will be heated faster than 65 otherwise would have been the case.

70 The speed of the conveyor is such that the pieces will be brought up to hot working or some other desired temperature by the time they fall from the holders 13 on discharge chute 15. For aluminum the hot working temperature will be in the neighborhood of 1000° F. and for brass in the neighborhood of 1500° F.

As soon as the hot pieces are contacted by the atmosphere, if they are heated to between 1000° F. and 1200° F., the carbon coating will disappear, apparently burned off, leaving the piece with its original surface. In those cases where the piece is heated to above 1200° F., the coating will burn off at about that temperature. By that time, however, an oxide will be formed on the surface so that the heating rate will not be substantially affected. When the pieces are heated below 1000° F., as will be the case with some types of aluminum, the coating may remain on the surface until positively removed. It has been found, however, that the coating serves as a lubricant in forging dies.

From the above it will be apparent that the method of this invention provides for what amounts to an automatic surface treatment of a slug or other piece to be heated, so that pieces, regardless of their initial surface condition, will be brought substantially to the same temperature in the same time. Such heating increases the efficiency of a production line forging operation, for example, by reducing individual treatment given to the various pieces and rejects due to improper heating. The method may also be used for the continuous heating of strip metal. In such case the heating time of a bright strip such as aluminum, brass or stainless steel is reduced, and the strip is evenly heated even though it may have dark streaks or spots on it.

While in accordance with the provisions of the statutes, I have illustrated and described the best form of embodiment of my invention now known to me, it will be apparent to those skilled in the art that changes may be made in the form of the apparatus disclosed without departing from the spirit and scope of the invention set forth in the appended claims, and that in some cases certain features of my invention may be used to advantage without a corresponding use of other features.

What is claimed is:

1. The method of heating uniformly to hot working temperature metal pieces having varying surface conditions which comprises:  
moving said pieces one after the other at a constant speed through a furnace having two adjoining chambers,  
heating the first chamber through which the pieces travel to a temperature above which fuel gas will crack,  
introducing fuel gas into said first chamber to crack the gas,

depositing a layer of carbon from the cracked gas on the surfaces of said pieces as they move through said first chamber,

heating the second chamber through which the pieces travel to a temperature sufficient to bring said pieces up to the desired hot working temperature by the time they leave said chamber, and

heating the carbon covered pieces in said second chamber to hot working temperature by radiation and convection heat whereby each piece, regardless of its original surface condition, will be heated to substantially the same temperature in substantially the same time as they leave said second chamber.

2. The method of heating metal pieces to hot working temperature which comprises moving the pieces through a furnace at a constant rate, creating in a first portion of the furnace through which the pieces pass a fuel gas rich atmosphere at a temperature sufficient to crack the gas, depositing carbon from the cracked gas evenly over the surface of the pieces in the first portion of the furnace, creating in the next portion of the furnace a temperature sufficient to heat the coated pieces to hot working temperature, and heating each of the pieces to substantially the same hot working temperature regardless of its original surface condition as it leaves the chamber.

3. The method of uniformly heating metal pieces having various surface characteristics which comprises moving said pieces one after the other through a path at a uniform speed, surrounding a first portion of said path with an atmosphere containing free fuel gas at a temperature sufficient to crack the gas, precipitating carbon from the cracked gas on the surface of the metal pieces to coat them uniformly with carbon, surrounding a second portion of said path with a temperature sufficient to heat said pieces to hot working temperature and heating said uniformly coated pieces in said second portion to substantially the same final desired temperature by the time they leave said second portion.

#### References Cited by the Examiner

##### UNITED STATES PATENTS

|           |         |          |       |            |
|-----------|---------|----------|-------|------------|
| 1,280,825 | 10/1918 | Pacy     | ----- | 148—20.3   |
| 2,051,828 | 8/1936  | Dester   | ----- | 148—20.3 X |
| 2,865,797 | 12/1958 | McCawley | ----- | 148—20.3   |
| 2,923,539 | 2/1960  | Meyer    | ----- | 75—5 X     |

DAVID L. RECK, Primary Examiner.